

1,279,720.

S. G. LEWIS.  
TENNIS RACKET AND THE LIKE.  
APPLICATION FILED DEC. 29, 1916.

Patented Sept. 24, 1918.

FIG.1.



FIG.2.



FIG.3.



WITNESSES

J. Herbert Bradley.  
Francis J. Townsend.

INVENTOR

Seneca G. Lewis  
by Christy & Christy  
his attorneys

# UNITED STATES PATENT OFFICE.

SENECA G. LEWIS, OF GREENSBURG, PENNSYLVANIA.

TENNIS-RACKET AND THE LIKE.

1,279,720

Specification of Letters Patent. Patented Sept. 24, 1918.

Application filed December 29, 1916. Serial No. 139,549.

To all whom it may concern:

Be it known that I, SENECA G. LEWIS, residing at Greensburg, in the county of Westmoreland and State of Pennsylvania, a citizen of the United States, have invented or discovered certain new and useful Improvements in Tennis-Rackets and the like, of which improvements the following is a specification.

10 My invention consists in a new article of manufacture: a tennis racket or like article of which the stringing consists of vegetable fiber coated with rubber.

In an application for Letters Patent of 15 the United States filed by me November 3, 1916, Serial No. 129,405, I have described and claimed racket stringing formed of catgut; the material now commonly used for the purpose, but catgut coated or sized with 20 rubber. And I now find that such coating or sizing makes possible the use of various materials not otherwise adequate as substitutes for the catgut. In a second and companion case to this, Serial No. 132,270, I describe and claim a racket stringing of rubber coated wire, and in this application I describe and claim a racket stringing of rubber-coated vegetable fiber. By virtue of a 25 rubber coating vegetable fiber becomes available to afford an adequate and durable racket-stringing material.

The vegetable fiber employed may be such as preferred, but ordinarily well made finely twisted cotton and linen cords will be found 30 to be most serviceable. The rubber may be applied as and after the manner described in my other applications referred to. It may be applied in the form of thin sheets or strips wrapped upon the completed cord or 35 upon the component strands of which the cord is ultimately composed; or it may, and preferably will, be applied by causing the cord (or the still unassembled strands) to pass through a liquid solution of rubber.

40 Since the fibrous cord or strand is porous, the rubber solution will not merely effect a coating but it will to some degree at least penetrate the fibrous substance, filling it and forming in consequence an integrated and 45 closely adhering coating. The solvent for the rubber in such a solution as is here contemplated may be such as is desired: bisulfite of carbon, chloroform, ether, naphtha or

another solvent. The strength of the solution and its fluidity or viscosity will be 50 adapted to afford a coating of desired penetration into the fiber and of desired thickness upon the cord or strand. As the coated cord or strand passes from the bath, it may 55 pass between wiping, spreading and compressing instrumentalities such as desired—between rolls, for example, or through a die-block. The cord or strand after being coated will preferably be disposed and supported in such position and arrangement and subjected to such conditions as to allow the rubber of the coating to become air-cured. And it will be understood that (air-curing being in contemplation) the initial rubber 60 preparation in solution (or in sheet form) 65 will be compounded with that end in view.

The so coated and cured article may be ready for application as stringing for 70 rackets and like articles, or it may be woven, twisted, wrapped, braided or otherwise combined with other strands, like itself or unlike, to produce the stringing desired.

My invention is illustrated in the accompanying sheet of drawings in which Figures 1 and 2 show two forms of rubber 80 coated vegetable fiber, and Fig. 3 shows a face view of a tennis racket equipped with my improved stringing.

In Fig. 1, the fiber 1 is provided with a rubbed coating in the form of a thin sheet 85 or strip wrapped upon the completed cord; while in Fig. 2 the rubber coating 3 is such as results from passing the cord through a liquid solution of rubber.

I have spoken of tennis rackets and like 90 articles, and in Fig. 3 I have shown a tennis racket 4. However in this phrase I mean to include rackets used in various games, lacrosse sticks, snow shoes, and other articles consisting of a frame and stringing drawn 95 taut upon it.

I claim as my invention:—

A tennis racket or like article consisting of a frame strung with a stringing of rubber-coated vegetable fiber.

In testimony whereof I have hereunto set my hand.

SENECA G. LEWIS.

Witnesses:

WALTER B. TOOLE,  
G. W. DUNN.